

Nov. 23, 1937.

F. W. HUMPHNER

2,100,140

DECALCOMANIA

Filed Jan. 15, 1936



Inventor:  
Ferdinand W. Humphner,  
By Chritton, Wiles, Davies, Hirsch & Dawson,  
Attest,

## UNITED STATES PATENT OFFICE

2,100,140

## DECALCOMANIA

Ferdinand W. Humphner, Oak Park, Ill., assignor,  
by mesne assignments, to Mid-States Gummed  
Paper Co., a corporation of Delaware

Application January 15, 1936, Serial No. 59,318

2 Claims. (Cl. 41—33)

This invention relates to a decalcomania and more particularly to a decalcomania which is engraved.

An object of the invention is to provide a decalcomania which is adapted to be used as a tax stamp, liquor label, revenue seal, etc., and which minimizes the possibilities of counterfeiting. A further object is to provide a decalcomania which is so prepared as to permit a steel engraved print 10 to be formed thereon. Other specific objects and advantages will appear as the specification proceeds.

The invention is illustrated in a preferred embodiment by the accompanying drawing in which is shown in perspective an enlarged view of the structure embodying my invention.

It is commonly known that a steel engraved print formed with certain shades of ink is practically impossible to counterfeit by photographic reproduction, or by other methods of counterfeiting. However, because of the peculiar character and construction of decalcomanias, I find that it is necessary to make certain changes and modifications to enable the steel engraving operation to be carried out effectively.

In the first place, the paper must contain enough moisture to withstand the impressions made by the steel die press and to permit the desired stretching of the paper under the pressure exerted. The paper should have the maximum of fiber bulk which will provide a cushion during the operation while also permitting movement of the fibers into the fine lines of a steel engraving without cutting of the paper base.

Preferably, the paper should be a loose, well-formed bulky sheet of unsized paper. I have found that a standard decalcomania finish, upon which very little pressure has been applied by calendering, or other means, is suitable. The paper may be coated with the usual starch coating and adhesive coating.

The adhesive may be of the usual type employed in decalcomanias. I have found it highly desirable, however, to add more than the normal amount of glycerine in the adhesive which provides the extra moisture needed to permit the maximum stretching of the paper. I also prefer

to add a vegetable wax, such as japan wax, to the adhesive to reduce tackiness in the adhesive.

After the base and the adhesive thereon have been prepared, as described above, the lacquer or ink film is formed on the adhesive. In view of the well-known method of forming decalcomania bodies by ink, it is believed unnecessary to describe the process. If the transfer body is formed by a lacquer, I prefer to use a lacquer which is flexible and yet which will retain its form when removed from the paper base so as to provide a satisfactory transfer body. The film of ink or lacquer laid on the adhesive should be of sufficient thickness to provide a removable and flexible film and also to receive the final imprint 15 of the steel die press.

While the paper takes the embossing of the steel die and shows the design on the paper side when it is submerged in water to release the film, the paper again takes its normal shape and the film is released, thus providing a steel die engraving decalcomania transfer for stamp purposes.

While in the foregoing description I have set forth certain preferred conditions, it will be understood that such preferred conditions are given 25 for the purpose of illustration and that many changes can be made without departing from the spirit of my invention.

The foregoing detailed description has been given for clearness of understanding only, and 30 no unnecessary limitations should be understood therefrom, but the appended claims should be construed as broadly as permissible, in view of the prior art.

I claim:

1. A decalcomania comprising: a paper base, a water-soluble adhesive thereon, said adhesive containing glycerine and vegetable wax, a transfer body on said adhesive, and a steel engraving print on the top of said transfer body.

2. A decalcomania comprising: a paper base, a water-soluble adhesive thereon, said adhesive containing glycerine and japan wax, a transfer body on said adhesive, and a steel engraving print on the top of said transfer body.

FERDINAND W. HUMPHNER.